

April 18, 1967

R. D. MCQUILLAN ET AL

3,314,784

COBALT-BASE ALLOY RESISTANT TO THERMAL SHOCK

Filed Nov. 21, 1963

3 Sheets-Sheet 1

THERMAL SHOCK DISTORTION OF COBALT-BASE ALLOYS  
CONTAINING Cr, W, and Ta.



*Fig. 1.*

INVENTORS  
ROBERT D. MCQUILLAN  
WILLIAM M. THOMAS  
ELMER L. FREY

BY *Frederick J. McCarthy, Jr.*

ATTORNEY

April 18, 1967

R. D. McQUILLAN ET AL

3,314,784

COBALT-BASE ALLOY RESISTANT TO THERMAL SHOCK

Filed Nov. 21, 1963

3 Sheets-Sheet 2



Fig. 2.

INVENTORS  
ROBERT D. McQUILLAN  
WILLIAM M. THOMAS  
ELMER L. FREY

BY *Frederick J. McCarty*

ATTORNEY

April 18, 1967

R. D. MCQUILLAN ET AL

3,314,784

COBALT-BASE ALLOY RESISTANT TO THERMAL SHOCK

Filed Nov. 21, 1963

3 Sheets-Sheet 3



Fig. 3.

INVENTORS  
ROBERT D. MCQUILLAN  
WILLIAM M. THOMAS  
ELMER L. FREY

BY *Frederick J. McCarthy Jr.*

ATTORNEY

# United States Patent Office

3,314,784

Patented Apr. 18, 1967

1

## 3,314,784 COBALT-BASE ALLOY RESISTANT TO THERMAL SHOCK

Robert D. McQuillan, William M. Thomas, and Elmer L. Frey, Kokomo, Ind., assignors to Union Carbide Corporation, a corporation of New York

Filed Nov. 21, 1963, Ser. No. 325,338  
11 Claims. (Cl. 75—171)

This invention relates to cobalt-base alloys for high temperature service and, more particularly, to alloys resistant to extreme conditions of high stresses and thermal shock.

Critical components of certain industrial equipment, such as machines or engines are subject to extreme conditions of heat, stresses, wear, erosion and the like. The so-called super-alloys have been developed to withstand these forces and cobalt-base alloys are particularly useful for this purpose. However, it is recognized that the usefulness of any component is ultimately determined by the capacity to withstand the total combined forces in the actual environment of operation.

One example of this situation exists with regard to alloys used in the vane section of a gas turbine engine. A particular prior art alloy hereinafter referred to as Alloy PA-I has been rather widely used in the manufacture of vanes of gas turbine engines. The nominal composition of PA-I alloy is 21 percent chromium, 10 percent tungsten, 0.9 percent carbon, 9.0 percent tantalum, 0.25 percent zirconium, up to 0.2 percent boron, and the balance cobalt, plus about 0.20 percent silicon, up to about 1 percent iron, and incidental impurities. This alloy has adequate strength to endure the stresses present in a vane component in gas turbine engines under many circumstances. However, it has been found that in actual operation in gas turbine engines, as a result of prolonged use, the vane components are detrimentally affected. For example, the components tend to become bowed or otherwise distorted due to the effect of thermal shock. Attempts to overcome this problem by minor compositional adjustments have proved to be unsuccessful.

There are other cobalt-base alloys known in the art that provide good service at temperatures up to about 1800° F. However, the known alloys have certain deficiencies principally in resistance to thermal shock, when in prolonged use at temperatures up to about 2000° F. Consequently there is an urgent need for new alloys that withstand the higher operating temperatures.

It is therefore an object of this invention to provide alloys for service up to about 2100° F., having the combined properties of high strength and thermal shock resistance.

Another object of this invention is to provide thermal shock-resistant cobalt-base alloys consisting essentially of cobalt, chromium, tungsten, tantalum and carbon as the effective alloying elements.

Other objects will be apparent from the following description and claims taken in conjunction with the drawing which shows:

In FIGURE 1, a graph illustrating the superior thermal shock resistance of alloys of the present invention.

In FIGURE 2, a photomicrograph (original magnification 200X) illustrating the microstructure of preferred alloys of the present invention.

In FIGURE 3, a photomicrograph (original magnification 200X) showing the microstructure of alloy PA-I.

An alloy in accordance with the present invention has a composition of 20 to 35 percent chromium, 5 to 20

2

percent tungsten, 3 to 5.5 percent tantalum, 0.7 to 1.3 percent carbon, balance cobalt and incidental impurities, the total chromium plus tungsten content of said alloy being greater than about 35 percent and not exceeding about 47.5 percent; the tungsten content being greater than about two times the tantalum content, the total chromium and tungsten content being between 8 and 12 times the tantalum content, and the tantalum being present in an amount less than any of the other metal alloying constituents.

Chromium, tungsten and tantalum are included in the allow of the present invention to provide the strength, corrosion and oxidation resistance, hardness and other properties necessary to resist high stresses at temperatures up to about 2100° F. and higher. Carbon must be present in the alloy to form the desired carbides. In order to provide the necessary control of the desired carbides, the carbon content must be restricted from about 0.70 to 1.3 percent and preferably within the range of 0.75 to 1.2 percent.

It has been discovered as part of the present invention that an extremely critical relationship must exist among the alloying metal elements chromium, tungsten and tantalum. The total chromium and tungsten content must be greater than about 35 percent but not exceed about 47.5 percent in the final alloy. Contents lower than about 35 percent yield an alloy markedly lower in strength while contents over about 47.5 percent tend to yield an alloy with undesirably low ductility. The tantalum content must always be the lowest of the three alloying metal elements. Also, the tungsten content must always be greater than about two times the tantalum content and the combined total chromium and tungsten content must be from about 8 to 12 times, and preferably about 10 times, the tantalum content.

A preferred practice of this invention is realized with alloys produced within the following compositional range in accordance with the aforescribed relationship.

|    |                  |                                     |
|----|------------------|-------------------------------------|
| 40 | Chromium         | 22.5 to 32.5 percent.               |
|    | Tungsten         | 8 to 18 percent.                    |
|    | Carbon           | .75 to 1.2 percent.                 |
|    | Tantalum         | 3 to 4.5 percent.                   |
| 45 | Ti, Zr, B        | Nil.                                |
|    | Other impurities | Low as possible and less than 5.5%. |
|    | Cobalt           | Balance.                            |

This preferred compositional range yields alloys that have an excellent combination of properties such as tensile and stress-rupture strength, ductility, oxidation resistance, thermal shock resistance and good castability characteristics.

The group of elements nickel, molybdenum, iron, silicon, columbium, manganese, and vanadium are at times adventitiously present in the raw materials used in preparing this class of cobalt base alloys. These elements, in small quantities, are not particularly harmful in the alloys of this invention, however, because their presence tends to dilute the effective elements and interfere with the relationship of the desired carbides in the structure, it is important that their content in the final alloy be limited to less than 4 percent nickel, less than 0.5 percent molybdenum, less than 2.5 percent iron, less than 0.5 percent silicon, less than 1.0 percent columbium, less than 0.5 percent manganese and less than 0.5 percent vanadium. The total content of these elements should not exceed about 5.5 percent and preferably is kept as low as possible in the final alloy.

Sulfur, magnesium, zirconium, nitrogen, boron and titanium should be kept below about 0.15 percent in the aggregate. The maximum individual contents for these

elements are 0.02%, 0.01%, 0.01%, 0.05%, 0.01% and 0.08% respectively. These foregoing elements in excessive amounts are particularly harmful in the alloy of this invention and reduce the resistance to thermal shock deformation and failure. Their presence can be minimized by various techniques such as (1) the proper choice of raw materials used in preparing the alloy, (2) preventing the inter-alloying of deoxidizers with the alloy, (3) the use of non-contaminated crucibles, molds and other materials that contact the molten alloy, and (4) using appropriate melting and casting processing steps, such as hereinafter described.

In this last respect, one unexpected advantage is realized in the processing of the alloy of this invention. For example, high-temperature alloys, now in use, often require a controlled content of one or more elements in the group, titanium, boron, zirconium, aluminum, magnesium and nitrogen. As a means of controlling the amount of these elements, it has been found necessary to melt and cast these alloys under a controlled atmosphere such as either an argon gas cover or in vacuum. Often a combination of both is required.

The alloy of the present invention does not require any of these elements in its composition. In fact, best results are obtained when the alloy is entirely free from these elements or at least contains less than about 0.15% in the aggregate. Therefore, there is no need for the extra processing steps involving atmosphere control. It has also been found that melting and casting in ambient air atmosphere yields the best results in the practice of the present invention since any minor amounts of titanium, zirconium, magnesium, aluminum, and nitrogen are practically or completely eliminated when the molten alloy is exposed to ambient atmosphere. In other words, a controlled atmosphere, i.e., vacuum and/or positive argon pressure, usually required for processing the prior art alloys, not only is not required, but actually may be detrimental in the processing of the alloy of the present invention.

To further illustrate the present invention the various alloys listed in Table I were prepared and tested.

TABLE I.—COMPOSITIONS OF TESTED COBALT-BASE ALLOYS

| Alloy No. | Weight Percent |       |      |      | Cr+W  | Cr+W,<br>Ta |
|-----------|----------------|-------|------|------|-------|-------------|
|           | Cr             | W     | C    | Ta   |       |             |
| 1         | 30.37          | 9.97  | 0.33 | 3.50 | 40.34 | 11.5        |
| 2         | 28.53          | 9.27  | 0.57 | 4.01 | 37.80 | 9.43        |
| 3         | 30.37          | 9.97  | 0.87 | 3.50 | 40.34 | 11.5        |
| 4         | 29.99          | 9.88  | 0.80 | 4.62 | 39.87 | 8.68        |
| 5         | 30.04          | 10.00 | 0.89 | 4.04 | 40.04 | 9.91        |
| 6         | 30.37          | 9.97  | 1.18 | 3.50 | 40.34 | 11.5        |
| 7         | 29.99          | 9.88  | 1.18 | 4.62 | 39.87 | 8.63        |
| 8         | 29.99          | 9.88  | 0.99 | 4.62 | 39.87 | 8.63        |
| 9*        | 31.78          | 9.05  | 0.46 | 4.03 | 40.83 | 10.40       |
| 10*       | 20.76          | 4.88  | 0.50 | 5.47 | 25.64 | 4.60        |
| 11        | 25.19          | 15.02 | 0.89 | 3.9  | 40.21 | 10.3        |
| 12        | 25.17          | 15.28 | 0.85 | 4.55 | 40.45 | 8.89        |
| 13        | 25.35          | 14.75 | 0.81 | 4.12 | 40.10 | 9.73        |
| 14        | 24.76          | 15.05 | 0.88 | 9.73 | 39.81 | 4.09        |
| 15        | 23.64          | 14.03 | 0.81 | 9.28 | 37.67 | 4.06        |
| 16        | 30.04          | 5.33  | 0.90 | 3.82 | 35.37 | 9.26        |
| 17        | 29.91          | 5.30  | 0.87 | 4.48 | 35.21 | 7.86        |
| 20        | 29.79          | 14.59 | 1.04 | 9.34 | 44.38 | 4.75        |
| 21        | 30.06          | 14.81 | 1.06 | 4.10 | 44.87 | 10.94       |
| 22        | 29.92          | 9.89  | 1.05 | 9.79 | 39.81 | 4.06        |
| 23        | 25.10          | 9.73  | 1.04 | 9.58 | 34.83 | 3.63        |
| 24        | 25.31          | 9.65  | 1.04 | 3.87 | 34.96 | 9.03        |
| PA-I*     | 21.00          | 10.00 | 0.9  | 9.0  | 31.00 | 3.44        |

\*Alloy 9 also contains 5.5 Mo, 3.45 Fe, and 2.90 Ni; Alloy 10 also contains 4.86 Mo and 2.66 Zr; Alloy PA-I also contains .25 Zr.

The melting of the alloys 1-24 was conducted in an induction furnace in an air atmosphere. Commercially available magnesium and alumina crucibles were used for melting alloys 1-24 and the melting practice to produce about 30 to 50 pounds of final alloy was the same for each of these alloys. This comprised charging the cobalt, tungsten, chromium and carbon into the induction furnace and melting in an air atmosphere at about 2700° 70 75

F. The melt was deoxidized with usual Ca Si deoxidizer and the tantalum was added to the melt; after interalloying the tantalum, the melt was again deoxidized with titanium. The temperature was then raised to about 2800° F. and the metal was cast into molds.

The PA-I alloy was melted and cast in a complex melting and casting furnace in a vacuum as is customary and required for this alloy in order to obtain optimum properties and also to control the zirconium content.

All of the alloys were cast in forms which provide specimens for various tests. In most cases, the cast specimens were in the form of turbine engine vane components in order to determine the characteristics of the alloy as regards the castability of a practical product. The alloy specimens were subsequently tested in the "as-cast" condition, i.e., no extra processing or heat treating steps were used or were necessary to obtain optimum properties. The test results shown in Tables II, III, IV, and V and the graph of FIGURE 1 show that alloys of the present invention (e.g. alloys 3, 4, 5, 11, 12, 13 and 21) provide a maximum resistance to thermal shock deformation and failure, yet the other required strength and endurance characteristics are better than, or at least comparable to, the known alloys now used in the art.

Alloy 24 of this invention, while not having as high a resistance to thermal shock deformation as the previously mentioned alloys 3, 4, 5, 11, 12, 13, and 21, nevertheless has a very good combination of mechanical properties and thermal shock resistance as shown in Tables II, III and IV.

TABLE II.—COBALT-BASE ALLOYS IN ORDER OF DECREASING RESISTANCE TO DISTORTION (THERMAL SHOCK RESISTANCE)

| Alloy No. | Deformation<br>after 500<br>Cycles, mils | Ratio of Carbide Formers |                    | Microstruc-<br>ture Type |
|-----------|------------------------------------------|--------------------------|--------------------|--------------------------|
|           |                                          | Cr+W, Ta                 | Carbon,<br>percent |                          |
| 21        | 3                                        | 10.94                    | 1.06               | A                        |
| 11        | 8                                        | 10.3                     | .89                | A                        |
| 12        | 8                                        | 8.89                     | .85                | A                        |
| 13        | 8                                        | 9.73                     | .81                | A                        |
| 3         | 11                                       | 11.5                     | .87                | A                        |
| 4         | 11                                       | 8.63                     | .80                | A                        |
| 5         | 11                                       | 9.91                     | .89                | A                        |
| 45        | 30                                       | 4.75                     | 1.04               | D                        |
| 20        | 30                                       | 4.06                     | 1.05               | C                        |
| 22        | 37                                       | 9.03                     | 1.04               | B                        |
| 24        | 52                                       | 3.63                     | 1.04               | C                        |
| 23        | 57                                       | 9.26                     | .90                | D                        |
| 16        | 57                                       | 7.86                     | .87                | D                        |
| 17        | 57                                       | 11.5                     | 1.18               | B                        |
| 6         | 57                                       | 8.63                     | 1.18               | B                        |
| 50        | 7                                        | 4.06                     | .81                | C                        |
| 15        | 61                                       | 8.63                     | .99                | E                        |
| 8         | 63                                       | 8.63                     | .88                | C                        |
| 14        | 79                                       | 4.09                     | .33                | D                        |
| 1         | 105                                      | 11.5                     | .57                | D                        |
| 2         | 135                                      | 9.43                     | .90                | F                        |
| PA-I      | 150                                      | 3.44                     | .50                | G                        |
| 10        | Over 150                                 | 4.69                     | .46                | H                        |
| 55        | 9                                        | Over 150                 | Over 150           |                          |

#### Description of microstructures by group

- 60 Group:
- A----- Microconstituents Continuous network of  $M_6C$  type carbides with little or no  $TaC$  present; uniform structure.
  - B----- Rich in  $TaC$ ,  $M_7C_3$  type carbides also present.
  - C----- Rich in acicular  $TaC$  with  $M_6C$  type carbides present.
  - D----- Rich in globular  $TaC$  with  $M_6C$  type carbides present.
  - E----- Rich in globular  $TaC$  with  $M_6C$  type carbides, and  $M_7C_3$  type carbides present.
  - F----- Zirconium nitrides and acicular tantalum carbides present; also massive  $M_6C$  carbide formation.

Group:

- G----- Microconstituents  
High content of zirconium nitrides  
and  $\text{Co}_2\text{W}$  compounds.
- H----- Carbides not continuous, massive  
columnar structure.

preferred process suggested herein and in accordance with the present invention were cast in the form of ingots which were subsequently hot worked and found to yield sound forgings. Compositional and hardness data for these alloys are shown in Table VI.

TABLE VI

|            | Composition, Weight Percent |       |      |     |      | Hardness, $\text{R}_c$ |        |
|------------|-----------------------------|-------|------|-----|------|------------------------|--------|
|            | Cr                          | W     | Ta   | C   | Co   | As-Cast                | Forged |
| Alloy 4-W  | 29.99                       | 9.88  | 4.62 | .80 | Bal. | 36                     | 49     |
| Alloy 13-W | 25.35                       | 14.75 | 4.12 | .81 | Bal. | 44                     | 49     |

TABLE III.—STRESS-RUPTURE DATA AT 2000° F. AND 2000 P.S.I.

| Alloy | Life, hours | Elongation, Percent | Reduction of Area, Percent |
|-------|-------------|---------------------|----------------------------|
| 2     | 7.0         | 9.0                 | 8.5                        |
| 3     | 14.5        | 22.0                | 38.0                       |
| 4     | 15.2        | 20.0                | 47.0                       |
| 6     | 13.4        | 15.1                | 20.0                       |
| 7     | 11.8        | 11.8                | 20.9                       |
| 9     | 1.9         | 11.0                | 18.2                       |
| 10    | 6.2         | 41.0                | 41.1                       |
| 11    | 33.5        | 5.5                 | 5.1                        |
| 12    | 27.1        | 8.0                 | 5.6                        |
| 13    | 17.4        | 13.5                | 17.6                       |
| 14    | 9.6         | 10.3                | 15.9                       |
| 16    | 28.5        | 6.4                 | 10.2                       |
| 21    | 11.3        | 8.9                 | 10.5                       |
| 22    | 5.3         | 18.7                | 28.8                       |
| 23    | 26.3        | 12.6                | 21.7                       |
| 24    | 40.9        | 7.6                 | 7.9                        |

TABLE IV.—AVERAGE ROOM TEMPERATURE TENSILE DATA FOR COBALT-BASE ALLOYS

| Alloy | Ultimate Tensile Strengths, X1,000 p.s.i. | Yield 2% Offset, X1,000 p.s.i. | Elongation, Percent | Reduction of Area, Percent |
|-------|-------------------------------------------|--------------------------------|---------------------|----------------------------|
| PA-I  | 135                                       | 100                            | 2.0                 |                            |
| 2     | 113                                       | 84                             | 3.1                 |                            |
| 5     | 130                                       | 93                             | 1.5                 | 5.0                        |
| 6     | 139                                       | 101                            | 1.5                 | 1.5                        |
| 9     | 120                                       | 95                             | 2.3                 | .8                         |
| 12    | 135                                       | 110                            | 2.0                 | 2.8                        |
| 14    | 120                                       | 109                            | 1.3                 | 2.0                        |
| 16    | 125                                       | 105                            | 2.3                 | .8                         |
| 21    | 147                                       |                                |                     | 3.1                        |
| 22    | 120                                       |                                |                     |                            |
| 23    | 148                                       |                                |                     |                            |
| 24    | 145                                       |                                |                     |                            |

TABLE V.—AVERAGE HIGH TEMPERATURE TENSILE PROPERTIES DATA

| Alloy | Temperature, ° F. | Ultimate Tensile Strengths, X1,000 p.s.i. | Yield 2% Offset, X1,000 p.s.i. | Elongation, Percent | Reduction of area, Percent |
|-------|-------------------|-------------------------------------------|--------------------------------|---------------------|----------------------------|
| 5     | 1,700             | 64                                        | 35                             | 14                  | 18                         |
| 5     | 1,900             | 38                                        | 19                             | 23                  | 30                         |
| 5     | 2,000             | 26                                        | 14                             | 36                  | 50                         |
| 12    | 1,700             | 75                                        | 44                             | 6                   | 12                         |
| 12    | 1,900             | 45                                        | 25                             | 14                  | 22                         |
| 12    | 2,000             | 33                                        | 18                             | 22                  | 33                         |
| PA-I  | 2,000             | 50                                        | 38                             | 10                  |                            |
| PA-I  | 1,700             | 30                                        | 25                             | 17                  |                            |
| PA-I  | 1,900             | 23                                        | 21                             | 20                  |                            |

Tables III, IV, and V particularly show that the alloys of the present invention in addition to having superior thermal shock resistance are at least comparable to, and in most instances substantially better than the other tested alloys as regards other mechanical properties.

It was also found that the alloys of this invention may be readily produced in the form of wrought products in addition to cast products. Two alloys prepared by the

Further tests which included a metallographic study of the tested alloys indicate that certain alloys of the present invention have a characteristic structure as compared to other alloys of this general class. The compositional range for these alloys is about 25-30% chromium, about 9.9-15% tungsten, about 3.5-4.6% tantalum, about 0.8-1.1% carbon, balance cobalt and incidental impurities the total chromium plus tungsten content of said alloy being greater than about 40 percent and not exceeding about 45 percent the tungsten content being greater than about two times the tantalum content, the total chromium and tungsten content being between 8 and 12 times the tantalum content, and the tantalum being present in an amount less than any of the other metal alloying constituents. For example, alloys 3, 4, 5, 11, 12, 13 and 21 shown in Table I which are within this range, have a very uniform continuous network of  $\text{M}_6\text{C}$  type carbides and are essentially free of TaC and the  $\text{M}_7\text{C}_3$  carbides. That is, 99 percent or more of the carbides are  $\text{M}_6\text{C}$ . This type of structure is identified as Type A in Table II and is shown in FIGURE 2 which is a photomicrograph (original magnification 200X) of alloy 4 of Table I having a composition of 29.99% chromium, 9.88% tungsten, 0.80% carbon, 4.62% tantalum, balance Co.

With reference to FIGURE 2, the continuous dark area indicated as 1 represents the  $\text{M}_6\text{C}$  carbide network and the white background area 3 is the metallic matrix of the alloy. The other alloys shown in Table II contain TaC and/or a high proportion of the  $\text{M}_7\text{C}_3$  type carbides; the identity of these structures are well known in the art and are described in Table II next to the corresponding alloy composition.

Further, by way of example, the microstructure of PA-I alloy is shown in FIGURE 3. This is identified as Type F in Table II. In FIGURE 3, massive  $\text{M}_6\text{C}$  carbide is shown at 5, acicular tantalum carbide is shown at 7 and zirconium nitride is shown at 9.

Tests results have also shown that a correlation appears to exist between the microstructure of the alloy and the terminal shock properties of the alloy. As shown in Table II, the best thermal shock resistance is obtained when the microstructure of the alloy is of the type shown in FIGURE 2 and identified as Type A in Table II.

The benefits which are characteristic of the alloys of the present invention are obtained by strict control of the proportion of carbide formers and carbon available in the total alloy, and it has been found that the combination of desired properties in the alloys of the present invention are obtained only when the composition of the alloy satisfies the following equation:

$$\frac{\text{Cr} + \text{W}}{\text{Ta}} = \frac{35 \text{ to } 47.5}{3 \text{ to } 5.5} = 8 \text{ to } 12$$

As previously noted it is further required that the carbon content be fixed within the range 0.70 to 1.3% and preferably 0.75 to 1.2% in order to obtain the desired

combination of properties. When carbon contents in alloys are outside of the limits of the present invention, suitable distribution and types of carbides are not formed. For example, Alloys 3, 4, 5, 11, 12 and 13 contain about 0.85% carbon with about 40% (Cr+W) and Alloy 21 contains 1.06% carbon with about 45% (Cr+W). Thus, the ratio of carbon to carbide formers remains about the same and these alloys have the desired combination of properties. On the other hand, alloys 1, 2, 6, 7 and others that contain carbon either above or below the suggested limits, while having apparently similar compositions to the aforementioned alloys do not have the same combination of mechanical strength properties.

Also as previously mentioned, the tantalum content is also critical in the alloys of this invention, since with alloys having less than about 3% tantalum, the corrosion resistance is marginal or inadequate. On the other hand, alloys containing more than about 5.5% tantalum contain undesirable amounts of acicular and/or globular tantalum carbides in their microstructure and consequently do not withstand the effects of thermal shock. By way of example, Alloys 12 and 14 are similar except for the tantalum content. However, alloy 12 with about 4.5% tantalum has excellent properties, whereas Alloy 14 with about 9.7% tantalum has inadequate resistance to thermal shock.

The data of Table II relating to distortion resistance (thermal shock resistance) were obtained by using test apparatus and test procedures well known in the art. Briefly the test used is as follows: Eight airfoil-shaped specimens are mounted on a hub, which rotates at 1725 r.p.m. and travels between a furnace and a water spray quenching station at preset time intervals. About 400 cc. of aspirated water is used as the quenching agent. Each cycle consists of 60 seconds exposure in the furnace, which operates at 2100° F., and 90 seconds cooling in the water spray. The specimens are heated to 2100° F. in the furnace in about 40 seconds. After each 100 cycles, the test is halted and the specimens are measured for deformation and are visually examined for cracking or other anomalies. Five hundred cycles constitute a complete test. Results of the test are graphically presented in FIGURE 1 and tabulated in Table II. FIGURE 1 shows the average deformation or bow of each specimen versus the number of cycles.

The deformation or bow is determined by the actual measured dimensional deviation from the original shape resulting from the thermal shock conditions of the test. The standard air-foil shaped specimens used in this test (one-inch width, two-inch length) are measured for deviation at 1.85 inches from the hub. FIGURE 1 clearly shows that the specimens made of alloys of this invention, alloys 3, 4, 5, 11, 12, 13, and 21 have much higher resistance to deformation resulting from thermal shock than the other tested alloys.

What is claimed is:

1. A thermal-shock resistant cobalt base alloy consisting essentially of 20 to 35 percent chromium, 5 to 20 percent tungsten, 3 to 5.5 percent tantalum, 0.7 to 1.3 percent carbon, a maximum of 0.08 percent titanium, a maximum of 0.01 percent zirconium, less than 1% columbium, balance cobalt and incidental impurities, the total chromium plus tungsten content of said alloy being greater than about 35 percent and not exceeding about 47.5 percent; the tungsten content being greater than about two times the tantalum content, the total chromium and tungsten content being between 8 and 12 times the tantalum content, and the tantalum being present in an amount less than the tungsten content and less than the chromium content.

2. An alloy in accordance with claim 1 wherein the carbon content is between about 0.75 and about 1.2 percent.

3. An alloy in accordance with claim 1 wherein the total chromium and tungsten content is about 10 times the tantalum content.

4. A thermal-shock resistant cobalt base alloy consisting essentially of about 25 to about 30 percent chromium, about 9.9 to about 15 percent tungsten, about 3.5 to about 4.6 percent tantalum, about 0.8 to about 1.1 percent carbon, a maximum of 0.8 percent titanium, a maximum of 0.01 percent zirconium, less than 1% columbium, balance cobalt and incidental impurities, the total chromium plus tungsten content of said alloy being greater than about 40 percent and not exceeding about 45 percent; the tungsten content being greater than about two times the tantalum content, the total chromium and tungsten content being between 8 and 12 times the tantalum content, and the tantalum being present in an amount less than the tungsten content and less than the chromium content said alloy being characterized by a microstructure having a substantially continuous network of carbides, at least 99% of said carbides being  $M_6C$  type carbides.

5. A thermal-shock resistant cobalt base alloy consisting essentially of about 30 percent chromium, about 10 percent tungsten, about 3.5 percent tantalum, about 0.9 percent carbon, a maximum of 0.08 percent titanium, a maximum of 0.01 percent zirconium, less than 1% columbium, balance cobalt and incidental impurities said alloy being characterized by a microstructure having a substantially continuous network of carbides, at least 99% of said carbides being  $M_6C$  type carbides.

6. A thermal-shock resistant cobalt base alloy consisting essentially of about 30 percent chromium, about 10 percent tungsten, about 4.6 percent tantalum, about 0.8 percent carbon, a maximum of 0.08 percent titanium, a maximum of 0.01 percent zirconium, less than 1% columbium, balance cobalt and incidental impurities said alloy being characterized by a microstructure having a substantially continuous network of carbides, at least 99% of said carbides being  $M_6C$  type carbides.

7. A thermal-shock resistant cobalt base alloy consisting of about 30 percent chromium, about 10 percent tungsten, about 4.0 percent tantalum, about 0.9 percent carbon, a maximum of 0.08 percent titanium, a maximum of 0.01 percent zirconium, less than 1% columbium, balance cobalt and incidental impurities said alloy being characterized by a microstructure having a substantially continuous network of carbides, at least 99% of said carbides being  $M_6C$  type carbides.

8. A thermal-shock resistant cobalt base alloy consisting essentially of about 25 percent chromium, about 15 percent tungsten, about 3.9 percent tantalum, about 0.9 percent carbon, a maximum of 0.08 percent titanium, a maximum of 0.01 percent zirconium, less than 1% columbium, balance cobalt and incidental impurities said alloy being characterized by a microstructure having a substantially continuous network of carbides, at least 99% of said carbides being  $M_6C$  type carbides.

9. A thermal-shock resistant cobalt base alloy consisting essentially of about 25 percent chromium, about 15 percent tungsten, about 4.6 percent tantalum, about 0.9 percent carbon, a maximum of 0.08 percent titanium, a maximum of 0.01 percent zirconium, less than 1% columbium, balance cobalt and incidental impurities said alloy being characterized by a microstructure having a substantially continuous network of carbides, at least 99% of said carbides being  $M_6C$  type carbides.

10. A thermal-shock resistant cobalt base alloy consisting essentially of about 25 percent chromium, about 15 percent tungsten, about 4.1 percent tantalum, about 0.8 percent carbon, a maximum of 0.08 percent titanium, a maximum of 0.01 percent zirconium, less than 1% columbium, balance cobalt and incidental impurities said alloy being characterized by a microstructure having a substantially continuous network of carbides, at least 99% of said carbides being  $M_6C$  type carbides.

11. A thermal-shock resistant cobalt base alloy consisting essentially of about 30 percent chromium, about 15 percent tungsten, about 4.1 percent tantalum, about 1.1 percent carbon, a maximum of 0.08 percent titanium,

a maximum of 0.01 percent zirconium, less than 1% columbium, balance cobalt and incidental impurities said alloy being characterized by a microstructure having a substantially continuous network of carbides, at least 99% of said carbides being  $M_6C$  type carbides.

## References Cited by the Examiner

## UNITED STATES PATENTS

2,974,036 3/1961 Thielemann ----- 75-171

3,118,763 1/1964 Thielemann ----- 75-171

## FOREIGN PATENTS

5 830,649 3/1960 Great Britain.  
838,835 6/1960 Great Britain.

DAVID L. RECK, Primary Examiner.

WINSTON A. DOUGLAS, Examiner.

C. M. SCHUTZMAN, R. O. DEAN, Assistant Examiners.